

Aug. 7, 1962

S. ILNYCKYJ ET AL  
ETHYLENE-VINYL ESTER POUR DEPRESSANT  
FOR MIDDLE DISTILLATES

3,048,479

Filed Aug. 3, 1959

6 Sheets-Sheet 1

FIGURE 1  
COPOLYMERIZATION OF ETHYLENE AND VINYL ACETATE



STEPHAN ILNYCKYJ  
CHARLES B. RUPAR INVENTORS

BY *W. O. T. Feilman*

PATENT ATTORNEY

Aug. 7, 1962

S. ILNYCKYJ ET AL  
ETHYLENE-VINYL ESTER POUR DEPRESSANT  
FOR MIDDLE DISTILLATES

Filed Aug. 3, 1959

3,048,479

6 Sheets-Sheet 2



STEPHAN ILNYCKYJ  
CHARLES B. RUPAR INVENTORS

BY *W. D. Telman*

PATENT ATTORNEY

Aug. 7, 1962

S. ILNYCKYJ ET AL  
ETHYLENE-VINYL ESTER POUR DEPRESSANT  
FOR MIDDLE DISTILLATES

3,048,479

Filed Aug. 3, 1959

6 Sheets-Sheet 3

FIGURE 3

EFFECT OF VINYL ACETATE CONTENT OF COPOLYMER



STEPHAN ILNYCKYJ  
CHARLES B. RUPAR INVENTORS

BY *W. O. T. Helm*

PATENT ATTORNEY

Aug. 7, 1962

S. ILNYCKYJ ET AL  
ETHYLENE-VINYL ESTER POUR DEPRESSANT  
FOR MIDDLE DISTILLATES

3,048,479

Filed Aug. 3, 1959

6 Sheets-Sheet 4

FIGURE 4

EFFECT OF VINYL ACETATE CONTENT ON POUR  
DEPRESSING POTENCY OF COPOLYMER



STEPHAN ILNYCKYJ  
CHARLES B. RUPAR INVENTORS

BY W. C. Kilman

## PATENT ATTORNEY

Aug. 7, 1962

S. ILNYCKYJ ET AL  
ETHYLENE-VINYL ESTER POUR DEPRESSANT  
FOR MIDDLE DISTILLATES

Filed Aug. 3, 1959

3,048,479

6 Sheets-Sheet 5

FIGURE 5  
EFFECT OF MOLECULAR WEIGHT OF COPOLYMER



STEPHAN ILNYCKYJ  
CHARLES B. RUPAR INVENTORS

BY *W. O. T. Helman* PATENT ATTORNEY

Aug. 7, 1962

S. ILNYCKYJ ET AL  
ETHYLENE-VINYL ESTER POUR DEPRESSANT  
FOR MIDDLE DISTILLATES

3,048,479

Filed Aug. 3, 1959

6 Sheets-Sheet 6

FIGURE 6  
POTENCY OF ETHYLENE POLYMERS AS POUR  
DEPRESSANTS FOR MIDDLE DISTILLATE FUELS



STEPHAN ILNYCKYJ  
CHARLES B. RUPAR INVENTORS

BY *W.C. Kelman*

PATENT ATTORNEY

# United States Patent Office

3,048,479

Patented Aug. 7, 1962

1

3,048,479

## ETHYLENE-VINYL ESTER POUR DEPRESSANT FOR MIDDLE DISTILLATES

Stephan Ilnyckyj and Charles B. Rupar, Sarnia, Ontario, Canada, assignors to Esso Research and Engineering Company, a corporation of Delaware

Filed Aug. 3, 1959, Ser. No. 831,244

6 Claims. (Cl. 44—62)

The present invention relates to improving the flow of low temperatures and the pour point characteristics of middle distillates. More particularly, the present invention relates to the preparation of improved low cold test hydrocarbon fuels, in particular heating oils and diesel fuels, kerosine, aviation turbo-jet fuels and other fuels that are subject to low temperatures.

The present application is a continuation-in-part of application Serial No. 719,188, filed March 5, 1958, entitled "Pour Depressant for Middle Distillates," now abandoned, for the same inventors.

With the increase in the use of hydrocarbon fuels of all kinds, a serious problem has arisen in areas frequently subjected to low temperatures in the cold characteristics of fuels. Particularly, serious problems have been encountered by heating oils and diesel and jet fuels that have too high a pour point, resulting either in distributional or operating difficulties or both. For example, the distribution of heating oils by pumping or syphoning is rendered difficult or impossible at temperatures around or below the pour point of the oil. Furthermore, the flow of the oil at such temperatures through the filters cannot be maintained, leading to the failure of the equipment to operate.

Also the low temperature properties of petroleum distillate fuels boiling in the range between about 250° and about 750° F. have attracted increasing attention in recent years because of the growth of markets of such fuels in subarctic areas and because of the development of turbo-jet aircraft capable of operating at altitudes where temperatures of —50° F. or lower may be encountered.

It is, of course, well known to add pour depressants to lubricating oils to lower the pour point. These lube oil additives, mostly high molecular weight organic compositions formed by alkylation of benzene or naphthalene or derivatives thereof or by polymerization of lower molecular weight methacrylates, or by condensation polymerization of various kinds, are not satisfactory in service with middle distillate and lighter fuels. Poor performance of these additives might possibly result from the structural differences between waxes occurring in lubricating oils and so-called middle distillates.

A wide variety of compounds have been found to be effective as pour point depressants for lubricating oil. Among the best known are "Paraflow," "Santopour" and "Acryloid" and their modifications. They are prepared either by condensing aromatic compounds with long chain paraffins, such as wax, or by condensing olefinic esters. It is generally considered that these pour depressants are effective in that in cooling an additive-containing oil, the hydrocarbon chain of the additive becomes incorporated into the crystal lattice of the separated wax, while the other part of the pour depressant molecule prevents the crystals from adhering together to form a gel structure. The failure of these additives to be effective in middle distillates may at least in part be due to the basic difference in the composition between the wax in lubricating oils and that in middle distillate fuels.

It is, therefore, the principal object of the present invention to set forth an improved pour depressant for middle distillate and lighter fuels. In general, these oils boil in the range from about 250° to 750° F.

2

It is a still further object of the present invention to provide heating oils, diesel fuel oils, kerosines and jet fuels having low pour points. Such fuels include aviation turbo-jet fuels, kerosines, diesel fuels, and heating oils. Aviation turbo-jet fuels in which the polymers may be used normally boil between about 250° and about 550° F. and are used in both military and civilian aircraft. Such fuels are more fully defined by U.S. Military Specifications MIL-F-5624C, MIL-F-25554A, MIL-F-25558A, and amendments thereto. Kerosines and heating oils will normally have boiling ranges between about 300° and about 750° F. and are more fully described in ASTM Specification D-396-48T and supplements thereto, where they are referred to as No. 1 and No. 2 fuel oils. Diesel fuels in which the polymers may be employed are described in detail in ASTM Specification D-975-35T and later versions of the same specification.

The polymeric pour depressants may, in accordance with the invention, be employed in conjunction with a variety of other additives commonly used in fuels such as those set forth above. Typical of such additives are rust inhibitors, anti-emulsifying agents, corrosion inhibitors, anti-oxidants, dispersants, dyes, dye stabilizers, haze inhibitors, antistatic agents and the like. It will frequently be found convenient to prepare additive concentrates for use in the various types of fuels and thus add all of the additives simultaneously.

Other and further objects of the present invention will appear more clearly hereinafter.

30 The pour depressant comprises ethylene-vinyl acetate copolymer. It is preferred that the parts by weight of ethylene in the copolymer be in the range from about 60 to 99% as compared to parts by weight of vinyl acetate in the range from about 40 to about 1%. A very desirable ethylene-vinyl acetate copolymer contains about 15 to 25% by weight of vinyl acetate, as for example, about 20% parts by weight of vinyl acetate.

35 The molecular weights of the ethylene-vinyl acetate copolymer are critical and should be in the range from about 1,000 to 3,000, preferably, in the range from about 1,500 to 2,200. The molecular weights are determined by K. Rast's method (Ber. 55, 1051, 3727 (1922)).

40 The ethylene-vinyl acetate copolymer as described above is used in a concentration in the range from about .001 to .5% by weight, preferably, in a concentration in the range from about .005 to .1% by weight.

45 Surprisingly, these low molecular weight copolymers have no effect upon the pour points of lubricating oils, thus emphasizing the difference in structure between the wax associated on the one hand with lube oils and on the other with middle distillates. The low molecular weight copolymers may be prepared by any peroxide process. In some instances, it may be desirable to first prepare a 50 higher average molecular weight polymerization product and then recover from that product material having a molecular weight within the range between about 1,000 and about 3,000. Since such polymerization products normally consist of a smear of polymers whose molecular weights vary over a wide range, an effective method for recovering the 1,000 to 3,000 molecular weight portion therefrom is to extract the product with a solvent such as normal heptane or methyl-ethyl ketone. Other methods for obtaining the low molecular weight materials 55 include thermal degradation of the high molecular weight polymer or treatment of the high molecular weight polymer with ozone in order to break the polymer chains. Still other methods also useful will be apparent to those skilled in the art.

60 A very desirable method is to conduct polymerization in a benzene solution using di-tertiary-butyl-peroxide as an initiator at a temperature in the range from about 280°

to 340° F. The preferred temperature is about 300° F. The pressure is in the range from about 700 to 2,000 pounds, preferably, at about 800 pounds. The autoclave or similar equipment containing the solvent, initiator and vinyl acetate is purged about three times with nitrogen, twice with ethylene and then charged with a sufficient amount of ethylene to yield the desired pressure when heated to the reaction temperature. During the polymerization additional ethylene is added whenever the pressure drops by about 100 p.s.i.g. Polymerization is considered complete when it is less than 50 p.s.i.g. pressure drop per hour. The product is stripped free of solid and unreacted vinyl acetate under vacuum.

A typical distillate fuel boiling in the range from 250° to 750° F. to which the present additives may be added are middle distillate heating oils. These fuels are of commercial grade and have typical properties as follows:

|                              |      |
|------------------------------|------|
| Composition:                 |      |
| Straight run gas oil         | 40   |
| Cat. cracked gas oil         | 60   |
| Inspections:                 |      |
| Gravity, ° API               | 29.1 |
| ASTM pour, ° F., no additive | +20  |
| Flash, Pensky-Martin, ° F.   | 192  |
| Distillation, ASTM, ° F.—    |      |
| I.B.P.                       | 398  |
| 10%                          | 492  |
| 50%                          | 566  |
| 90%                          | 612  |
| F.B.P.                       | 644  |

The improvements obtained by adding the additives in accordance with the present invention are set forth in the following table. All pour points quoted hereafter were obtained by ASTM Method D-97-47.

A number of tests were conducted using various polymers in a 50-50 blend of virgin gas oil and cracked gas oil. The virgin gas oil boiled in the range from about 350° to 700° F., and the cracked gas oil boiled in the range from about 350° to 650° F. The blend had a pour of +20° F. The various polymers were prepared under varying pressure and other varying operating conditions. As pointed out heretofore, the critical factors with respect to desirable polymers are molecular weights and the concentration of the vinyl acetate in the polymer. The results of these tests are shown in the following table:

40%, the effectiveness of the additive is greatly decreased (runs No. 9 and 10).

Reference is made of FIGURE 1 which shows that at a constant pressure, the percentage of vinyl acetate in the copolymer increases with increasing concentration of this chemical in the solvent. The copolymerization was carried out at a pressure of 750 p.s.i.g., at a temperature of 300° F., utilizing benzene as a solvent and di-tertiary-butyl-peroxide as the initiator.

Reference is made to FIGURE 2 which illustrates that at a constant concentration of vinyl acetate in the solvent, the ratio of vinyl acetate in the polymer decreases with increasing partial pressure of ethylene. The concentrations of the vinyl acetate utilized in the solvent were: 0.2 wt. percent; 2.1 wt. percent and 6.3 wt. percent. Other conditions were identical with those specified with respect to FIGURE 1.

Reference is made to FIGURE 3 which shows the potency of the copolymers as pour depressants for middle distillates. The middle distillate was identical with that specified with respect to Table I. Curves A, B, C, D, E and F correspond to run Nos. 9, 10, 2, 3, 1 and 13, respectively of Table I. It is to be noted that curve F, containing about 20% of vinyl acetate was very effective.

Reference is made to FIGURE 4. This figure illustrates the relationship of the potency of the pour depressants to their vinyl acetate content. Curve A contains .05% pour depressant, whereas, curve B contains 0.1% pour depressant. It is to be noted that the most potent pour depressant was obtained at 850 p.s.i.g. when the copolymer contained about 80% ethylene and 20% vinyl acetate. It is to be noted from FIGURE 4 that copolymers containing more than 20% vinyl acetate show a drop in pour depressing activity. This is particularly pronounced at lowe concentration of the additive. At 0.05% concentration, the activity of pour depressants becomes negligible when the copolymer contains about 24% of vinyl acetate. At 0.1% concentration, the copolymers show some pour depressing activity until the vinyl acetate amounts to about 35% of the total polymer.

Reference is made to FIGURE 5 which illustrates the effect of pressure at which the copolymer is produced on its activity as pour depressants. The polymers obtained at pressures lower than about 600 p.s.i.g. show little promise as pour depressants. As the molecular weight is proportional to pressure during the synthesis, this illus-

TABLE I  
*Synthesis of Copolymers of Ethylene and Vinyl Acetate*

[Conditions of polymerization: 300° F., di-tert-butylperoxide initiator, benzene solvent]

| Run No. | Vinyl Acetate Conc., Wt. Percent |            | Pressure, p.s.i.g. | Yield grams per gram Peroxide | ASTM Pour Point, <sup>1</sup> ° F. |      |       |      |
|---------|----------------------------------|------------|--------------------|-------------------------------|------------------------------------|------|-------|------|
|         | in Benzene                       | in Product |                    |                               | 0.05%                              | 0.1% | 0.25% | 0.5% |
| 1       |                                  | 7.5        |                    |                               | 0                                  | -25  | -50   | -40  |
| 2       | Ni1                              | Ni1        | 750                | 19                            | +5                                 | 0    | -25   | -70  |
| 3       | .53                              | 3.0        | 750                | 18                            | +5                                 | 0    | -50   | >-70 |
| 4       | 2.1                              | 8.4        | 750                | 17.5                          | 0                                  | -10  | >-70  | >-70 |
| 5       | 8.5                              | 28.1       | 750                | 22.5                          | +10                                | -25  | >-70  | >-70 |
| 6       | 2.1                              | 5.8        | 900                | 23                            | 0                                  | -20  | >-70  | -60  |
| 7       | 2.1                              | 17.9       | 400                | 9                             | +15                                | +10  | +10   | 0    |
| 8       | 2.1                              | 12.1       | 600                | 14                            | +15                                | +5   | -15   | -70  |
| 9       | 21.0                             | 53.8       | 750                | 31                            | +20                                | +20  | +20   | +10  |
| 10      | 14.8                             | 44.7       | 750                | 26                            | +15                                | +15  | +10   | +10  |
| 11      | 11.7                             | 35.2       | 750                | 23.5                          | +10                                | +10  | -60   | -70  |
| 12      | 6.3                              | 24.3       | 750                | 18                            | +10                                | -50  | >-70  | -60  |
| 13      | 6.3                              | 20.4       | 850                | 23                            | -40                                | >-70 | >-70  | -40  |
| 14      | 6.3                              | 14.7       | 1,600              | 29.5                          | -10                                | >-70 | >-70  | >-70 |

<sup>1</sup> 50/50 Blend of Virgin Gas Oil and Cat. Cracked Gas Oil, ASTM Pour +20° F.

From the above, it is apparent that 3% vinyl acetate is much superior to an ethylene polymer containing no vinyl acetate in the monomer (run No. 3 vs. run No. 2). It is also apparent that a concentration of vinyl acetate approximately of 28% is very effective (run No. 5), and that when the vinyl acetate concentration exceeds about

70% the copolymer must have a certain minimum molecular weight to be effective as pour depressants.

Reference is made to FIGURE 6 which illustrates the effectiveness of the copolymer of the present invention as a pour depressant of polyethylene polymers. All polymers used had a molecular weight of about 1,300.

The pour depressant for middle distillate fuels has little effect on oil viscosity, particularly in the concentration ranges in which it is effective. This is clearly shown in Table II.

TABLE II

*Effect of Ethylene Vinyl Acetate Copolymer on Pour Point and Viscosity of Light Gas Oil*

[ASTM pour point of the oil:  $+25^{\circ}\text{ F.}$ ]

| Weight Percent Ethylene Copolymer (1) | Pour Point Depression, $^{\circ}\text{ F.}$ | Viscosity of Oil $100^{\circ}$ , SUS |
|---------------------------------------|---------------------------------------------|--------------------------------------|
| 0.01                                  | 0                                           | 38.27                                |
| 0.03                                  | 20                                          | 33.21                                |
| 0.05                                  | 50                                          | 33.30                                |
| 0.1                                   | 65                                          | 33.24                                |
| 0.3                                   | 80                                          | 33.36                                |
| 1.0                                   | 55                                          | 33.54                                |
|                                       | 5                                           | 39.37                                |

(1) 800 molecular weight as determined by Rast Method.

It is also of interest to note that with as little as 1% of the additive, the effectiveness in depressing pour is considerably less than it is in smaller dosages, i.e., about 0.1%. This adverse effect of polyethylene-vinyl acetate copolymer pour depressant at higher concentrations is believed to result from the tendency of this polymer to form a gel structure with the oil on cooling when present in sufficient quantities.

A large number of other polymers were investigated for their middle distillate pour point depression properties. None were effective for this purpose, as shown in Table III.

TABLE III

*List of Hydrocarbons Found Ineffective as Pour Depressants for Middle Distillates*

| Hydrocarbon                                | Wt. Percent in oil | Pour Depression, $^{\circ}\text{ F.}$ | Remarks                               |
|--------------------------------------------|--------------------|---------------------------------------|---------------------------------------|
| <b>Microcrystalline Waxes:</b>             |                    |                                       |                                       |
| M.P. $180^{\circ}\text{ F.}$               | 0.001              | 2                                     |                                       |
|                                            | 0.01               | 1                                     |                                       |
|                                            | 0.1                | -6                                    |                                       |
|                                            | 1.0                | -8                                    |                                       |
| M.P. $183^{\circ}\text{ F.}$               | 0.001              | 0                                     |                                       |
|                                            | 0.01               | -6                                    |                                       |
|                                            | 0.001              | -1                                    |                                       |
|                                            | 0.01               | -2                                    |                                       |
|                                            | 0.1                | -5                                    |                                       |
|                                            | 1.0                | -10                                   |                                       |
| M.P. $115^{\circ}\text{ F.}$               | 0.001              | -3                                    |                                       |
|                                            | 0.01               | -2                                    |                                       |
|                                            | 0.1                | -7                                    |                                       |
|                                            | 1.0                | -11                                   |                                       |
| <b>Visc. 100, SUS</b>                      |                    |                                       |                                       |
| Polypropylenes                             | 0.1                | 20                                    | 34.9                                  |
|                                            | 0.1                | 2.5                                   | 42.80                                 |
|                                            | 0.1                | 2.5                                   | 118.9                                 |
|                                            | 0.1                | 2.2.5                                 | 563.0                                 |
|                                            | 0.1                | 2.2.5                                 |                                       |
| n-C <sub>7</sub> sol. linear Polypropylene | 0.2                | +2.5                                  |                                       |
|                                            | 0.5                | +2.5                                  |                                       |
|                                            | 1.0                | +12.5                                 | Solid, Mol. Wt. Range, 10,000-30,000. |
|                                            | 2.0                | 2.5                                   |                                       |
| <b>Polybutenes ("Indopol"):</b>            |                    |                                       |                                       |
| "L-10"                                     | 0.1                | +2.5                                  | -65 330                               |
| "L-50"                                     |                    | 0                                     | -35 420                               |
| "L-100"                                    | 0.1                | +5                                    | -25 470                               |
| "H-35"                                     | 0.1                | 0                                     | 0 660                                 |
| "H-50"                                     | 0.1                | +2.5                                  | +5 700                                |
| "H-100"                                    | 0.1                | 0                                     | +20 780                               |
| "H-300"                                    | 0.1                | +5                                    | +35 940                               |

TABLE III.—Continued

| Hydrocarbon                                             | Wt. Percent in oil | Pour Depression, $^{\circ}\text{ F.}$ | Remarks                                       |
|---------------------------------------------------------|--------------------|---------------------------------------|-----------------------------------------------|
| Polybutene-1                                            | 0.1                | +5                                    | Low Visc. Oil.                                |
|                                                         | 0.5                | 0                                     | Do.                                           |
|                                                         | 0.1                | +2.5                                  | Do.                                           |
|                                                         | 0.1                | +7.5                                  | Visc. at $100^{\circ}\text{ F.}$ , 1,269 SUS. |
| <b>Visc. at <math>100^{\circ}\text{ F.}</math>, SUS</b> |                    |                                       |                                               |
| Polybutene-2                                            | 0.1                | +5                                    | 54.0                                          |
|                                                         | 0.1                | +5                                    | 78.10                                         |
|                                                         | 0.1                | 0                                     | 841.2                                         |
|                                                         | 0.1                | +2.5                                  | 1,493.0                                       |
| Polyisobutylene:                                        | 0.001              | 0                                     |                                               |
| Mol. Wt. 23,400                                         | 0.001              | +3                                    |                                               |
|                                                         | 0.1                | 0                                     |                                               |
|                                                         | 1.0                | 0                                     |                                               |
| Mol. Wt. 100,000                                        | 0.001              | 0                                     |                                               |
| Mol. Wt. 200,000                                        | 0.001              | 0                                     |                                               |
| Mol. Wt. 300,000                                        | (3)                | 0                                     |                                               |
| Polycyclopentane                                        | 0.1                | 0                                     | Visc. at $100^{\circ}\text{ F.}$ , 6,340 SUS. |

NOTE.—Polystyrenes—None of several grades tried was soluble in oil.

(1) (+) Pour Depression.

(-) Pour Elevation.

<sup>2</sup> Liquid.

<sup>3</sup> Insoluble in Oil.

It has hitherto been pointed out that wax in middle distillate fuels is different from wax in lubricating oils, and that pour depressant additives effective in one case are ineffective in the other. In Table IV below, two common lubricating oil pour depressants, namely, "Paraflo" and "Acryloid" are compared with ethylene polymer having a molecular weight of about 1750.

TABLE IV

*Effect of Various Additives on ASTM and Stable Pour Points of a 356° to 682° F. Virgin Gas Oil*

| Additive                                                      | Weight Percent | ASTM Pour, $^{\circ}\text{ F.}$ |
|---------------------------------------------------------------|----------------|---------------------------------|
| None                                                          |                | +25                             |
| "Paraflo"                                                     | 0.2            | +20                             |
|                                                               | 0.5            | +15                             |
| "Acryloid"                                                    | 1.0            | +5                              |
|                                                               | 0.2            | +15                             |
|                                                               | 0.5            | +10                             |
|                                                               | 1.0            | 0                               |
| Ethylene Vinyl Acetate Copolymer (Mol. Wt. 1750) <sup>1</sup> | .05            | -40                             |
|                                                               | .1             | <-70                            |
|                                                               | .25            | <-70                            |
|                                                               | .5             | -40                             |

(1) As determined by Rast Method.

55 These data clearly demonstrate the superiority of the low molecular weight ethylene-vinyl acetate copolymers over the lubricating oil pour depressants. On the other hand, when these copolymers are added to lubricating oils, they in turn are ineffective.

TABLE V

| Weight Percent Copolymer (Mol. Wt. 800) | ASTM Cloud/Pour, $^{\circ}\text{ F.}$ |                     |                     |
|-----------------------------------------|---------------------------------------|---------------------|---------------------|
|                                         | MCT-10 <sup>1</sup>                   | MCT-30 <sup>1</sup> | MCT-60 <sup>1</sup> |
| None                                    | +10/+5                                | +30/+30             | +36/+35             |
| 0.1                                     | +28/-15                               | +32/+30             | +50/+45             |
| 0.5                                     | +48/+15                               | +40/+25             | +56/+40             |

<sup>1</sup> Paraffinic type obtained from Leduc crude by distillation, dewaxing, phenol extraction and clay treatment.

It is probable that the different effects of these copolymers on pour of lubricating oils is due at least in part to the structural differences between waxes in middle

distillates (n-paraffins) and dewaxed lubricating oils (iso-paraffins and naphthenes).

Not all oils are equally responsive to the additive. Catalytically cracked gas oil is considerably more responsive than a virgin gas oil. Both, however, are improved in pour point, as shown in Table VI.

TABLE VI  
*Response of Virgin and Cracked Gas Oil to Polyethylene Vinyl Acetate Copolymer Pour Depressant*  
[Av. mol. wt.—800<sup>1</sup>]

| Type of Gas Oil              | Copolymer Wt. Percent | ASTM Pour °F. | Stable Pour, °F. |
|------------------------------|-----------------------|---------------|------------------|
| Virgin <sup>2</sup>          | {Nil<br>0.1           | +25<br>+0     | +15<br>+5        |
| Cat. Cracked <sup>3</sup>    | {Nil<br>0.1           | +10<br>-84    | +5<br>-35        |
| 50% Virgin, 50% Cat. Cracked | {Nil<br>0.1           | +15<br>-40    | +10<br>-35       |

<sup>1</sup> As determined by Rast method.

<sup>2</sup> Boiling range 442–674° F.

<sup>3</sup> Boiling range 394–638° F.

<sup>4</sup> Less than.

The effectiveness of the low molecular weight ethylene-vinyl acetate copolymers as pour depressants for jet fuels is shown in Table VII below. Jet fuels are subject to extreme temperature conditions, and it is highly important that they have low pour and freezing points. For comparison are shown values of customary pour depressants such as "Paraflo," a condensation product of chlorinated wax and naphthalene; "Acryloid," a polymer of methyl methacrylate; and "OA-142," a copolymer of alkyl fumarate and vinyl acetate. Jet fuels are selected hydrocarbon fractions boiling in the naphtha and kerosene boiling range.

TABLE VII  
*Pour Depressants for Jet Fuels*

|                                      | Pour Point, °F. | Freezing Point (FSM), °F. |
|--------------------------------------|-----------------|---------------------------|
| Jet Fuel                             | -65 to -70      | -57.5                     |
| Jet Fuel + 5% Copolymer <sup>1</sup> | <-110           | -60                       |
| Jet Fuel + 1% Copolymer              | -95             | -58                       |
| Jet Fuel + .05% Copolymer            | -90             | -60                       |
| Jet Fuel + .025% Copolymer           | -80             | -59                       |
| Jet Fuel + .0125% Copolymer          | -75             | -59                       |
| Jet Fuel + 1% Paraflo                | -95             | -58                       |
| Jet Fuel + 5% Paraflo                | -85             | -                         |
| Jet Fuel + 25% Paraflo               | -65             | -                         |
| Jet Fuel + 1% Paraflo                | -75             | -66                       |
| Jet Fuel + .05% Paraflo              | -75             | -                         |
| Jet Fuel + .025% Paraflo             | -68             | -                         |
| Jet Fuel + .0125% Paraflo            | -65             | -56                       |
| Jet Fuel + 1% Acryloid               | -75             | -                         |
| Jet Fuel + .75% Acryloid             | -70             | -                         |
| Jet Fuel + 5% Acryloid               | -65             | -                         |
| Jet Fuel + .25% Acryloid             | -65             | -                         |
| Jet Fuel + 12.5% Acryloid            | -70             | -                         |
| Jet Fuel + 1% OA-142                 | -70             | -                         |
| Jet Fuel + .5% OA-142                | -75             | -                         |
| Jet Fuel + 25% OA-142                | -75             | -                         |
| Jet Fuel + 12.5% OA-142              | -75             | -                         |

<sup>1</sup> 800 Molecular Weight as determined by Rast Method.

The effectiveness of the present ethylene-vinyl acetate copolymers with respect to increasing filterability is shown

by the following table. Various percentages of different substances were added to a heating oil and the filterability determined by the Hagemann and Hammerich Test reported in DIN-51770 (Bestimmung der Filtrierbarkeit von Diesel Kraftstoffen). A 40 mesh screen was employed.

TABLE VIII

|                                                                       | ° F. |
|-----------------------------------------------------------------------|------|
| Base oil                                                              | +25  |
| 10 +0.5% Acryloid                                                     | +15  |
| +2.0% Paraflo                                                         | -28  |
| +0.1% Ethylene-vinyl acetate copolymer (molecular weight about 1,000) | -37  |

What is claimed is:

1. A petroleum distillate fuel composition having an improved pour which comprises essentially a petroleum distillate fuel having a boiling range between about 250° F. and about 750° F. which has been improved with respect to pour point by the incorporation therein of a pour depressing effective amount in the range from about .001 to .5% by weight of an oil soluble copolymer of ethylene and a vinyl fatty acid ester having from about 3 to about 5 carbon atoms in the ester, said copolymer having a molecular weight in the range from about 1000 to 3000, said copolymer being further characterized by containing from about 15 to 25% by weight of said vinyl fatty acid ester.
2. A petroleum distillate composition having an improved pour which comprises essentially a petroleum distillate fuel having a boiling range between about 250° F. and about 800° F. which has been improved with respect to pour point by the incorporation therein of a pour depressing effective amount in the range from about .01 to about 0.25% by weight of an oil soluble copolymer of ethylene and a vinyl fatty acid ester having from about 3 to about 5 carbon atoms in the ester, said copolymer having a molecular weight in the range from about 1000 to 2500, said copolymer being further characterized by containing from about 15 to about 28% by weight of said vinyl fatty acid ester.
3. Fuel composition as defined by claim 1 wherein said vinyl ester is a vinyl acetate.
4. Fuel composition as defined by claim 3 wherein said copolymer is present in a concentration from about .005 to 0.1%.
5. A fuel composition as defined by claim 1 wherein said copolymer has a molecular weight between about 1,600 and about 2,000 and wherein said copolymer is present in a concentration from about .005 to 0.1% by weight.
6. Fuel as defined by claim 1 wherein said copolymer is a copolymer of ethylene and vinyl acetate wherein the copolymer contains about 20% by weight of vinyl acetate.

References Cited in the file of this patent

UNITED STATES PATENTS

|           |                 |               |
|-----------|-----------------|---------------|
| 2,327,705 | Frolich et al.  | Aug. 24, 1943 |
| 2,499,723 | Coffman et al.  | Mar. 7, 1950  |
| 2,657,188 | Dennison et al. | Oct. 27, 1953 |
| 2,746,925 | Garber et al.   | May 22, 1956  |
| 2,800,401 | Lusebrink       | July 23, 1957 |